

Oct. 12, 1943.

F. L. SIMONS

2,331,575

SAFETY PAPER AND METHOD OF MAKING SAME

Filed Aug. 3, 1940

*Fig. 1.*



*Fig. 2.*



*Fig. 3.*



INVENTOR

*Francis L. Simons*  
BY

*Kenyon & Kenyon*  
ATTORNEYS

## UNITED STATES PATENT OFFICE

2,331,575

SAFETY PAPER AND METHOD OF MAKING  
SAME

Francis L. Simons, Montclair, N. J., assignor to  
George La Monte & Son, Nutley, N. J., a corporation of New Jersey

Application August 3, 1940, Serial No 350,423

13 Claims. (Cl. 117—1)

This invention relates to safety paper and method of making same.

It is a purpose of this invention to afford a safety paper that has the capacity to reveal attempts to erase by mechanical erasure legends written thereon. It is a special advantage of safety paper embodying this invention that it is adapted to evidence attempted alteration of legends written thereon in pencil.

Ordinary pencil markings or legends that have been applied to paper as by handwriting in pencil thereon are readily erasable by mechanical erasure, there being a variety of erasing compositions, generally made up in a rubber base, that are suitable for erasing pencil markings. Most writing pencils are made up with a small eraser of this type at the end thereof.

Attempts have heretofore been made to make pencil legends more difficult to erase by providing so-called "indelible" pencils that include a lead containing a coloring material that strikes into the paper and is very difficult to erase.

According to the present invention a paper is afforded which when written upon with a pencil of the usual type will reveal any attempts to remove the pencil marking by mechanical erasure.

It is a feature of this invention that a suitable base sheet is provided with a coating of substantial thickness that overlies a surface of the base sheet, and that some coloring material such as a dye is carried by the surface of the coating without penetrating therethrough. The material of the coating is of any suitable color, preferably white or nearly so, and the color of the coloring material is of a contrasting color. The coating material while carrying the color of the coloring material at the surface therefor comprises a substantial portion that is uncolored by said coloring material.

When a paper constituted as above described is written upon with a pencil, the pencil forms a clearly inscribed legend of the usual character. If attempt is made to erase the pencil legend by mechanical erasure, however, the mechanical erasure tends to rub off the dye or other coloring matter that is superficially carried by the coating so that wherever the mechanical erasure occurs the contrasting color of the underlying body of the coating material e. g. white, becomes more prominent thereby clearly evidencing the attempted erasure. It is very difficult if not impossible to replace color of the coloring material that has been removed by the mechanical eras-

sure so that the attempted alteration of the paper can not be detected.

In such paper the coating composition is preferably of a character to be described below that tends to receive the pencil marking so that considerable mechanical erasure is required to remove the pencil legend and so that removal of the pencil legend by mechanical erasure will also remove the coloring material to a very pronounced degree.

The advantages of a safety paper of the character described are several. It is often desirable to use a pencil instead of pen and ink in making notations and legends on paper, which legends should be protected from attempted alteration. An example of this character is afforded by dining checks which after the figures giving the amount due have been filled in are used by the waiter in making change to be returned by the waiter to the customer. Such dining checks, if of the ordinary type that can readily be altered can be used by dishonest waiters in a fraudulent way. It is highly desirable that such dining checks be adapted to reveal any attempted alterations of pencil legends inscribed thereon. Use of pencil safety paper for dining checks is only one of many uses to which safety paper embodying this invention may be put.

For the purpose of illustrating the practice of this invention and affording a better understanding thereof it will be described in connection with certain specific examples thereof and in connection with the accompanying drawing, wherein

Fig. 1 is a cross section of a portion of a sheet of safety paper embodying this invention on a very greatly enlarged scale.

Fig. 2 is a plan view of a sheet of safety paper embodying this invention, illustrating the effect of mechanical erasure thereon, and

Fig. 3 is a largely diagrammatic sectional elevation of suitable means for applying the coloring material.

In Fig. 1 the pencil safety paper comprises a sheet 10 of paper of any desired type and thickness. Usually the paper runs from about .002 to .025 inch in thickness, i. e. from paper that is quite thin to paper having sufficient body to be somewhat boardy in character. The paper may be writing paper, book paper, tag board, box board, card board, bristol board or the like and is preferably not a highly absorptive type of paper. Somewhat more generally the term paper is used in a broad sense as covering sheet material of the character aforesaid or other similar

or equivalent sheet material suitable for inscription of legends in pencil thereon when treated according to this invention.

Overlying the paper 10 is a coating 11, which, for purposes of exemplification may for example be composed of English china clay and casein as a binder. This composition may contain about 100 parts of the clay to each 15 parts of casein together with a minor proportion of some alkaline material such as tri-sodium phosphate, sodium carbonate or the like to render the casein water soluble. An exemplary formula for a suitable coating composition and a description of the manner of application of the coating will be given more in detail below. The coating is preferably applied so as to be uniformly of substantial thickness and so as to have a matte or eggshell surface.

Overlying the coating 11 is a layer 12 of a suitable coloring material such as Methylene Blue, for example, the color of which is different from the color, e. g. white, of the underlying coating material. The dye adheres to the outside surface of the coating as a very thin deposit. In this connection the layers shown in Fig. 1 are not drawn to scale inasmuch as the relative thickness of the layer 12 has been exaggerated for clarity in the showing in the drawing. As a matter of fact the layer 12 of coloring material is an extremely thin superficial deposit.

The layer 12 of coloring material may be deposited uniformly over the entire surface of the coating 11 or non-uniformly. In Fig. 2 the coloring 12 is shown in the form of a plurality of parallel lines of dye separated by undyed portions. Alternatively the lines could be separated by intervening areas which are of less color intensity.

In Fig. 2, the effect of a mechanical erasure is illustrated. On the face of the pencil safety paper the legend 1 2 3 4 5 6 7 appears and is to be regarded as having been placed thereon by pencil handwriting. If attempt is made to erase the figures 6 and 7 from the legend the effect of the erasure is that shown in Fig. 2. At and adjacent the figures 6 and 7 of the legend the coloring material 12 has been rubbed off so that instead of the blue colored lines or other surface coloring of the paper a white area appears that is in sharp contrast to the color of the remainder of the paper and clearly indicates the attempted alteration. The faint outline of the figures 6 and 7 may still be visible as shown in Fig. 2. This is in accordance with the normal action of the pencil safety paper. The action of the pencil in inscribing the legend in the safety paper tends to abrade the surface coating somewhat and colored material from the lead pencil tends to work into the coating so that it is quite difficult to remove by mechanical erasure. Thus, upon attempt to remove a pencil legend from the face of the safety paper, a faint outline of the original legend usually remains in the local area from which coloring material has been removed thereby enhancing the tell-tale evidence of attempted alteration.

The manufacture of the paper may be exemplified as follows. An aqueous binder solution may be made up containing 100 pounds of casein, 5 pounds of borax, 6.5 pounds of tri-sodium phosphate and 2 gallons of 26° ammonia together with water to form 100 gallons. The binder component, namely the casein, therefore is present in such amount that each gallon of solution contains 1 pound of casein. English china clay is incorporated in the binder solution, about 100

pounds of the clay being employed for each 15 pounds of casein. This coating mixture is applied to a paper sheet or web so that the paper will carry about 5 to 8 pounds of the casein and clay mixture (dry weight) per ream of paper measuring 17 x 22 inches.

The application of the coating may be made in a variety of different ways. For example the coating can be applied by a brush coater, an application of the coating composition carried by the paper web being spread uniformly by a plurality of oscillating brushes. Alternatively the coating can be applied by a roll coater, an application of the coating composition carried by the paper web being spread uniformly by rapidly rotating rolls between which the paper passes. United States patents, Nos. 1,597,218 and 1,597-219, may be cited as illustrative, of a suitable roll coater. An air brush coater may also be used, an application of the coating composition carried by the paper being spread uniformly by a blast of air. United States Patent No. 1,980,923 is illustrative of an air brush coater. The coating may also be applied by a cast coating operation wherein the coating material is dried while in contact with a smooth surface as described in United States Patent No. 1,719,166. The coating material may also be applied during the manufacture of the paper. Thus paper from a paper machine, after it has been partially dried may be passed through a roll coater, the drying of the paper being completed thereafter. United States patents, Nos. 1,707,333; 1,921,369; and 2,044,281 illustrate the application of coatings in this way. Alternatively the coating may be applied while the paper is still on the screen of a Fourdrinier machine, the paper thereafter being made up and finished in the usual way, and for such an operation reference may be made to United States Patent No. 2,079,846. A still further method of application consists merely in passing paper during the manufacture thereof through a tub-size bath, the paper carrying the coating composition being finished in the usual way.

After the coating material has been applied in any of the ways mentioned above by way of example, the paper is subjected in subsequent treatments only to light calendering which leaves the coating with a light matte or eggshell finish. Preferably the coated paper is passed through a super-calender and whose rolls are entirely unweighted.

The paper which has been coated as above described is then passed through a bath of coloring material e. g. a dye bath. In its simplest form this can be done merely by passing a web of the paper carrying the superficial coating through a dye bath, removing excess solution and drying the paper thus treated.

In Fig. 3 is shown a simple type of apparatus that may be used to apply the coloring material. The dye solution 13 is contained in a tank 14. A web 16 of the paper that has been coated and dried is taken from the roll 15 and is submerged in the bath 13 by causing it to pass under the roller 17. The web carrying the dye solution is then passed between pressure rolls 18 and 19. The roll 18 may be embossed with a suitable design while roll 19 may be plain. The paper web is subjected to pressure e. g. about 100 pounds to about 250 pounds per inch of line contact between the rolls, and since the recesses 20 on the surface of roll 18 prevent paper underlying the recesses from being compressed, portions only of the web are subjected to the pres-

sure. The portions of the web subjected to the pressure take up more of the dye in the dye bath than the other portions of the surface of the web. After being subjected to pressure between rolls 18 and 19 the web is again submerged in the bath 13 by causing it to pass under roller 21 and upon emerging from the bath is passed between the wringer rolls 22. The paper web thereafter is passed to a plurality of drying rolls 23 which may be heated and is subjected to drying until it contains about 6% of moisture.

The result of the foregoing operation is to color the surface of the coating material that overlies the surface of the paper. The coating material is of high white color substantially throughout and the dye occurs only at the surface of the coating so that the body of the coating remains uncolored. The dye is distributed over the entire surface of the coating but whenever the pressure is applied by the embossed roll 18 the coloration is more pronounced so that the surface of the paper is colored with two shades of the same color. The pattern of the two shades is determined by the embossing on the roll 18. The pattern may be in the form of parallel lines, reticulated lines, portions in the form of a seal, etc. as may be desired. The occurrence of the dye in an overall pattern or design of different shades of the same color applied to the surface of the coating is to be preferred in the practice of this invention.

In the above described apparatus rolls 18 and 19 may be omitted so that the coated paper may merely be immersed in the dye bath and then passed between wringer rolls 22 to remove excess of the dye solution before the paper is dried. In such case the coating will receive an overall application of dye that is of substantially uniform color intensity throughout.

In addition to the foregoing any other means for applying the dye to the coated paper as a thin application or layer deposited on the surface of the coating may be employed such as spray application, printing operation, calender staining or the like.

Referring to the specific coating composition above described other alkaline materials may be used with the casein binder such as triethanolamine, sodium silicate, lime, caustic soda or the like adapted to cause the casein to occur in soluble form.

In addition to casein other binder materials may be used for the coating. For example one pound of glue dissolved in one gallon of water affords a suitable binder solution which can be used with a filler such as china clay. Likewise starch made up with 1 pound per gallon of water affords a desirable binder solution. Shellac may also be used 1 pound being dissolved per gallon of water with the aid of a little borax or ammonia. Albumen e. g. egg albumen may also be used as a binder. Such binders are either white or substantially colorless or are only lightly colored so that in combination with white or light colored pigments, a coating composition that is white or nearly so is produced. By reference to a coating composition, filler, pigment or the like as being light colored, any material which is white or approximately white is intended.

The filler that is used may likewise be varied. English china clay or its American equivalent is very satisfactory. English china clay is selected primarily because of its whiteness. The only requirements of the clay for the coating are

that it be high white in color and of sufficient degree of fineness to be free from grit and also be well washed so as to be free from impurities such as soluble electrolytes or iron.

5 Another example of a satisfactory filler is satin white which is a mixture of precipitated calcium sulphate and aluminum hydroxide. Blanc fixe, which is a mixture of precipitated barium sulphate and aluminum hydroxide, is also desirable. Other examples of suitable fillers are precipitated chalk (calcium carbonate), titanium dioxide, zinc sulphide, asbestos, lithopone, etc.

While the foregoing filler materials may be used separately they may be mixed together 15 and it is usually preferable to do so as a better coating composition is afforded thereby. For example English china clay mixed in about equal proportions with satin white or blanc fixe affords a very desirable filler.

20 In addition to the foregoing other filler materials may also be used. The foregoing fillers have a high white color and are desirable for this reason inasmuch as it is usually desirable to have the coating that is carried by the paper as white as possible. If the coating may be of some other color than white then fillers having colors other than white may be employed. In this connection many clays, especially of a reasonably light color may be used as well as other filler materials that are sufficiently finely-divided 25 not to result in an excessively gritty coating for the paper. Use of mineral fillers is desirable inasmuch as mineral fillers do not have a pronounced affinity for the coloring matter thereby minimizing the tendency of the coloring matter to penetrate substantially into or through the coating composition.

The amount of filler that is used in proportion to a binder material such as casein, glue, starch, shellac or the like is preferably about 15 to 40 parts 30 of the binder for each 100 parts of filler. The optimum amount in any case will depend upon the filler selected and type of binder material. A filler such as china clay can be used in relatively high proportion e. g. about 100 parts of china clay to about 15 parts of binder. When satin white is used it is usually desirable to employ more of the binder, e. g. about 35 parts of binder to 100 parts of the satin white. In general it is desirable to employ enough binder to hold the filler in place so that it will not easily rub off, avoiding any excess of binder, on the other hand, that would impart excessive glossiness to the coating material as applied. Depending upon the filler and binder being used, and upon the mechanical coating method, the final coating mixture may require more or less thinning with water so as to obtain a good working consistency.

60 In applying the coating composition by immersion in a size-tub it is desirable to keep the filler material in suspension so that the coating will be applied uniformly to the paper. The presence of a protective colloid is desirable in keeping the filler in suspension. When the binder is an organic colloid such as starch, glue, casein, or the like such binder material being colloidal will in itself act as a protective colloid. Other protective colloid materials may also be incorporated in the suspension of filler such as methyl cellulose, pectin, etc.

70 In order to promote the occurrence of the filler in a state of suspension in the composition it is also desirable to employ a wetting agent of which many are known such as sulphonated lauryl alcohol, sulphonated cetyl alcohol, certain sulfo-

nium compounds, e. g. those described in United States Patent No. 2,192,906, various diamides, e. g. those described in United States Patent No. 2,193,963 or the like. The presence of the wetting agent is not essential but is desirable in achieving uniformity of application of the coating composition in the practice of this invention.

The coating material is applied to the paper so that preferably about 5 to 8 pounds of the coating composition by dry weight per ream of sheets 17 x 22 inches will be deposited upon the paper. While lesser amounts may be used it is not regarded as desirable to have deposited on the paper less than 2 pounds per ream of sheets 17 x 22 inches. While the coating can be applied so that it will be in excess of 8 pounds per ream of sheets 17 x 22 inches the additional thickness of coating material ordinarily serves no useful purposes according to this invention and may make the paper excessively bulky.

The amount of the coating composition that is employed is of considerable importance inasmuch as the coating composition serves to cover the fibers of the paper sheet (e. g. the sheet 10 in the foregoing example) so that when the dye material is applied the dye will not strike through to the fibers. Heretofore it has been the practice in applying a dye to a sheet of paper to cause the dye to penetrate to substantial depth and special liquid vehicles and wetting agents have been used for this purpose. By way of contrast according to the present invention sufficient coating material is caused to overlie the paper so that the dye in the dye bath is prevented from contacting the fibers of the paper and preferably the dye from the dye bath merely adheres to the surface of the coating composition. Penetration of the coating by the dye is reduced to a minimum and preferably does not occur to any substantial extent. The coating material carrying a dye or the like only at the surface is to be distinguished from a coating material that is colored throughout the thickness thereof.

The texture of the coating composition is such that it will readily receive legends inscribed in pencil thereon. To this end the mineral filler materials especially hard abrasive filler materials have a somewhat abrasive action on pencil lead causing the particles of lead abraded from the pencil to be received by the coating composition and become embedded therein. Moreover, by providing the coating with a matte or eggshell finish instead of a glossy surface the reception of legends applied by a lead pencil is facilitated. As aforesaid the lead from a lead pencil appears to work into the coating so as to be quite difficult to remove. From this point of view it is desirable that the coloring material be as readily removable by mechanical erasure from the paper coating as pencil legends that may be inscribed thereon. Preferably, the coloring material is more readily removable by mechanical erasure from the coating composition than any pencil inscriptions applied to the coating composition so that the removal of the coloring material will be very apparent upon mechanical erasure sufficient to result in any substantial removal of a pencil legend inscribed on the paper.

The pencil that is used in inscribing a legend on the pencil safety paper may be an ordinary lead pencil which produces a grey or nearly black marking depending upon whether the pencil is "hard" or "soft." The pencil safety paper is also adapted for use with other types of pencil, e. g.,

colored pencils. The only limitation in this regard is that the color of the coloring material applied to the surface of the coating should be different in color or color intensity from the color of the pencil so that the legend will show up when inscribed on the paper.

While this invention has been described hereinabove primarily from the point of view affording a safety paper that is adapted to evidence attempted mechanical erasure of legends written thereon in pencil, it is apparent that safety paper embodying this invention is likewise adapted to evidence attempted mechanical erasure of legends written on the paper in other ways. Thus, for example, safety paper embodying this invention is adapted to reveal attempted mechanical erasure of legends written thereon by typewriter. The safety paper of this invention is likewise adapted to reveal attempted mechanical erasure of legends in the form of so-called carbon copies produced by writing with a pencil, a typewriter or the like on a first sheet and transmitting the writing to an underlying sheet by means of carbon paper or the like interposed between the first sheet and the underlying sheet on which the carbon copy is produced. With regard to legends written in writing ink on safety paper embodying this invention, the superficially colored coating material comprising a filler and a binder readily receives ink, and the ink when applied is very difficult to remove either by mechanical or chemical erasure and any attempted mechanical erasure will be evidence in the manner above described.

35 The coloring matter or dye that is used in the coloring bath may vary widely depending primarily upon the color desired. For most purposes, basic dyes are regarded as preferable. Examples of such dyes are Methylene Blue, Methyl 40 Violet, Malachite Green, Bismarck Brown, Saffranine, Rhodamine, etc.

45 Acid dyes may also be used, such as Buffalo Blue Black, Blue Black SX, Acid Green LX, Acid Violet, Croceine Scarlet, etc.

50 The foregoing dyes are fugitive dyes that can be decolorized by application of a chemical ink eradicator in the form of a chemical oxidizing agent such as dilute hypochlorite solutions (e. g., a 2% solution of sodium hypochlorite) or permanganate solutions (e. g., a 1% solution of potassium permanganate). When such dyes are used, the safety paper will evidence attempted erasure, either by mechanical erasure or by use of a chemical ink eradicator.

55 Other dye materials which may be used in the pencil safety paper but which are not sensitive to chemical ink eradicators, are Naphthol Green, Palatine Fast Yellow, Palatine Fast Orange, and New Red B. Dyes such as these are mentioned in 60 order to illustrate the fact that the paper of this invention is designed primarily as a pencil safety paper without regard to whether or not the coloring matter that is used is sensitive to chemical ink eradicators. When it is said herein and in the claims that a dye is carried by the surface of the coating of coating material that in turn is adherent to a paper base sheet, it is to be understood that the dye is carried superficially as 65 a stain on the surface of the coating, and that no binder vehicle for the dye is present. As is the practice in the dyeing or staining of materials, the dye is applied in an aqueous solution that does not contain a binder vehicle, and this is 70 to be distinguished from the formulation of

paints, lacquers, printing inks and the like, which consist essentially of a coloring agent such as a pigment together with a binder vehicle such as drying oil, resinous material or the like.

While reference has been made to applying to one side only of a web or sheet of paper a coating composition which carries only at the surface coloring material readily removable by mechanical erasure, it is apparent that both sides of the web or sheet may be treated to afford pencil safety characteristics in the practice of the invention. Moreover, it is to be understood that the specific embodiments of this invention herein described have been set forth merely for the purpose of exemplifying the practice of this invention and that the exemplary embodiments may be varied considerably within the scope of this invention as defined in the following claims.

I claim:

1. A safety paper adapted to evidence mechanical erasure of a legend written thereon, said safety paper comprising a base sheet, a coating of substantially white coating material which comprises substantially white mineral filler pigment and binder material that bonds said filler pigment to said base sheet as an adherent coating and which coating material is applied substantially uniformly to a surface of said base sheet so as to weigh at least about 2 pounds per ream of sheets 17 x 22 inches, and a dye that is superficially carried by the outer surface of said coating material without a binder vehicle and that does not penetrate through said coating material to said paper and that is readily removable by mechanical erasure to render more prominent the white color of said coating material.

2. A safety paper according to claim 1 wherein said dye is a basic dye.

3. A safety paper adapted to evidence mechanical erasure of a legend written thereon, which safety paper comprises a paper base sheet, a coating of light colored coating material applied to a surface of said base sheet so as to weigh about 2 to approximately 8 pounds per ream of sheets 17 x 22 inches, said coating material consisting essentially of inorganic filler sufficiently finely-divided not to impart grittiness to the coating and a binder that bonds said filler to said base sheet as an adherent coating adapted for the inscription of a legend thereon and containing about 15 to about 40 pounds of said binder for each 100 pounds of said filler, and a dye that is carried by the surface of said coating as a stain deposited from solution without a binder vehicle and that does not penetrate said coating to substantial depth and that normally masks the light color of said coating material and is adapted to be readily removed from said surface of said coating upon mechanical erasure so as to expose the light color of said coating.

4. A method of making safety paper which comprises applying to the surface of paper a coating material comprising a finely-divided mineral filler and a binder adapted to bond said filler to said surface to form a coating weighing at least 2 pounds per ream of sheets 17 x 22 inches and suitable for the inscription of a legend thereon, and applying an aqueous solution of a dye to the surface of the coating, the paper being subjected to pressure in local areas of predetermined design to cause the dye solution to be absorbed to greater degree where said pressure is applied, thereby producing a paper having a design distinguished by areas of different intensity of the same color, the dye solution not

penetrating through the coating in any of said areas and not containing a binder vehicle and said dye as thus applied to the surface of said coating being readily removable by mechanical erasure to expose underlying coating material uncolored by said dye.

5. A safety paper adapted to evidence mechanical erasure of a legend written thereon, which safety paper comprises a paper base sheet, a coating that is superficially applied to surface of said base sheet and that comprises a finely-divided inorganic filler pigment and a binder that bonds said filler pigment to said base sheet as an adherent coating suitable for the inscription of a legend thereon, said coating material being applied substantially uniformly to said base sheet so as to weigh at least about 2 pounds per ream of sheets 17 x 22 inches, a dye that is carried by the outer surface of said coating without a binder vehicle and that does not penetrate said coating to substantial depth, said dye being of a substantially different color from the color of said coating and being readily removable from the surface of said coating upon mechanical erasure so as to expose the contrasting color of said coating.

6. A safety paper according to claim 5 wherein said dye is fugitive dye adapted to be decolorized by a chemical ink eradicator, thereby affording a safety paper that is adapted to evidence attempted erasure either by mechanical erasure or by use of a chemical ink eradicator.

7. A safety paper adapted to evidence mechanical erasure of a legend written thereon, which safety paper comprises a paper base sheet, a coating of substantial thickness of coating material that is applied so as to overlie a surface of said base sheet and that comprises inorganic filler which is sufficiently finely-divided not to impart grittiness to the coating and which imparts to the coating a matte upper surface and a binder which bonds said inorganic filler to said base sheet as an adherent coating adapted for the inscription of a legend thereon, said coating material being applied substantially uniformly to said base sheet so as to weigh at least 2 pounds per ream of sheets 17 x 22 inches, and a dye that is superficially carried by said coating without a binder vehicle and that does not penetrate substantially into said coating or to said base sheet, said dye being of a substantially different color from the color of said coating material and being readily removable by mechanical erasure to render more prominent the color of said coating material.

8. A safety paper according to claim 7 wherein said dye is applied so as to form a predetermined overall pattern defined by areas of different color intensity.

9. A safety paper adapted to evidence mechanical erasure of a legend written thereon, which safety paper comprises a paper base sheet, a coating of light-colored coating material that is adapted for the inscription of a legend thereon and that is applied substantially uniformly to a surface of said base sheet so as to weigh at least about 5 pounds per ream of sheets 17 x 22 inches, said coating material consisting essentially of finely-divided inorganic filler which is the preponderant constituent of the coating material and a binder which bonds said inorganic filler to said surface of said base sheet as an adherent coating, and a dye that contrasts with the light color of said coating material and that is carried by the surface of said coating without a binder

vehicle and that does not penetrate substantially into said coating material, said dye being readily removable from the surface of said coating by mechanical erasure, so as to expose the light color of said coating material.

10. A method of making safety paper which comprises applying to the surface of paper a coating material comprising a finely-divided mineral filler and a binder adapted to bond said filler to said surface to form a coating weighing at least 2 pounds per ream of sheets 17 x 22 inches and suitable for the inscription of a legend thereon, and applying to the surface of the coating an aqueous solution of a dye having a color different from the color of said coating, the dye solution not penetrating through the coating and not containing a binder vehicle, and said dye thus applied to the surface of said coating being

readily removable by mechanical erasure to expose underlying coating material uncolored by said dye.

11. A method according to claim 10 wherein 5 said coating after application to said paper is subjected to light calendering to provide a matte surface.

12. A method according to claim 10 wherein 10 said coating material comprising said filler and said binder is applied to said paper in the form of an aqueous composition containing a wetting agent.

13. A method according to claim 10 wherein 15 said coating material comprising said filler and said binder is applied to said paper in the form of an aqueous composition containing a protective colloid.

FRANCIS L. SIMONS.